

## UNITED STATES PATENT OFFICE

FRANK O. KICHLIN, OF LEBANON, PENNSYLVANIA, ASSIGNOR TO BETHLEHEM STEEL COMPANY

## MANUFACTURE OF LOW-CARBON CHROME STEEL

No Drawing.

Application filed April 20, 1926. Serial No. 103,377.

This invention relates to the manufacture of ferro-chromium alloys and is more particularly directed to the manufacture of chrome steels of low carbon content and of 5 chrome irons containing a substantial proportion of chromium.

The desirable rust-resisting property of low carbon chrome steel and chrome iron is well known, but hitherto the high cost of 10 manufacture, due to the necessity of using ferro-chromium of very low carbon content for alloying with low carbon steel, has prevented the wider use of such compositions. When ferro-chromium is obtained by the carbo-reduction of chrome ores, it is impossible 15 to avoid the inclusion of carbon in the ferro-alloy, and this residual carbon is normally removed by subsequent refining operations, which involve losses in chromium, as for example by bessemerizing the alloy. Ferro-chromium of low carbon content may also 20 be obtained by well known aluminothermic methods, but the cost of the thermic reagent is prohibitive in a ferro-alloy for use in a 25 commercial steel.

An object of this invention is, therefore, a 30 method of manufacture, whereby low carbon chrome steel or chrome iron may be obtained without having recourse to expensive refining operations, nor to expensive raw materials.

A further object of this invention is the 35 direct utilization of pig iron, whether itself containing chromium or not, with chrome ore for the production of chrome steel and iron.

A further object of this invention is to effect 40 the decarburization of pig iron, of steel or of ferro-alloys by the addition of ore in a more effective manner than has hitherto been attainable.

With these objects in view, the invention 45 consists in reducing chrome ore with the carbon normally contained in blast furnace pig iron, in such a manner that an intimate contact is effected between the metallic oxides of the ore and the carbon of the pig iron, so that the carbon at a suitable temperature, such as may be obtained in an electric furnace, reduces the metallic oxides of the ore 50 in substantially equivalent proportions and

is replaced in the pig iron by the metals reduced from the ore.

Heretofore, attempts to introduce an alloying element, as for example chromium, into a bath of steel by the addition of an ore of the 55 alloying element, have not been economically successful. Operating difficulties are introduced when the ore addition amounts to a substantial proportion of the total furnace charge, as would be the case if a high content 60 of the alloying element were desired. With chrome ore these difficulties are principally due to the fact that the chromic oxide of the ore addition has the effect of stiffening the slag and rendering it impossible to effect any 65 substantial alloying of the chromium with the metal of the bath. The addition of fluxes to maintain the proper fluidity of the slag is limited by the consequent increase in slag volume, which for practical reasons must not 70 exceed a definite proportion of the furnace capacity.

I have discovered that these difficulties may be entirely overcome, by effecting contact between the pig iron and the chrome ore, when 75 both components are in substantially comminuted condition. The pig iron may be obtained in a suitable state of comminution, by granulating it from its molten condition in the well known manner; while the ore may be 80 crushed to the size desired in any convenient manner.

Preferably, I granulate molten pig iron by rapidly cooling a spray of molten metal. This granulation may be carried out directly 85 when tapping a blast furnace charge, or the pig iron may be melted in a special cupola and granulated therefrom. In order to insure constant conditions in the subsequent furnace operations, it may be advantageous 90 to classify the granules in batches of approximately similar particle size. I also crush the chrome ore to a size that will allow of its intimate mixture with the granulated pig iron. A furnace charge is made up by mixing a convenient quantity of the granulated pig iron with an amount of crushed chrome ore, the metallic oxides of which are in substantial excess of the amount required to 95 combine with the carbon in the pig iron, and 100

with the necessary quantity of lime. This charge is melted in an electric furnace, the temperature of which is maintained at a point suitable for the reduction of chromium and at the end of the heat I obtain a chrome steel, having a content of chromium commensurate with the carbon originally present in the pig iron, and which is itself substantially carbon free. It will be understood that the refining operations for removing undesirable impurities from steel, normally practiced in a basic electric furnace under a lime slag, may be carried out if desired, subsequently to the reducing and decarburizing operation above described. Obviously in order to avoid the necessity of an extensive refining of the fusion bath, and consequent loss of time thereby, I prefer to utilize for my furnace charge a pig iron having a low content of these impurities.

For the purposes of my invention, I have found that pig iron derived from chromiferous iron ores, as for example the Mayari ores of Cuba, are particularly suitable, since the chromium content of the pig iron can thereby be profitably utilized, serving to increase the content of chromium in the alloy above that obtainable by the carbo-reduction of the chrome ore. In the same manner, by using a pig iron containing another alloying element besides chromium, as for example nickel, I can introduce this second alloying element into the final product in a simple and economical manner.

The following example will illustrate in a comprehensive manner the practice of my invention in a case where it is desired to manufacture a low carbon chrome steel, containing also an appreciable percentage of nickel. The known methods of manufacture would involve the reduction of chrome ore and the subsequent laborious decarburization of the ferro-chromium obtained, or alternatively the expensive alumino-thermic reduction of chrome ore; in either case a low carbon ferro-chromium, preferably as low as one tenth of one per cent. carbon, is essential if a low carbon alloy steel is desired. For the same reason, carefully selected low carbon steel scrap would be melted to form the fusion bath, and after the usual refining steps for phosphorus and sulphur the necessary quantity of the aforesaid low carbon ferro-chrome would be added to the bath and alloyed therewith, after which nickel would be introduced by an appropriate addition of nickel plaquettes.

In my process, I take, for example, a chromiferous pig iron, such as that derived from the Mayari ores of Cuba, having the following analysis: carbon 3.99, manganese 0.79, phosphorus .073, sulphur .014, silicon 0.40, nickel 0.89 and chromium 2.72. I granulate this pig iron by melting it and pouring the molten stream into cold water, and select

sixty pounds of the granulated material of approximately similar particle size. I mix with the granulated iron, one hundred pounds of chrome ore, having a chromic oxide content of about 43%, and crushed to suitable mesh, and also sixty pounds of lime. This mixture is then charged into an electric furnace and melted, the necessary additions of fluorspar being made as required. The reaction between the carbon of the pig iron and the oxides of the ore proceeds smoothly and without involving the production of excessive, nor of viscous, slag. The product obtained has the following composition: carbon 0.14, manganese 0.08, phosphorus 0.044, sulphur 0.015, silicon 0.014, nickel 0.94, chromium 12.39.

From the above it will be evident that I have devised a cheap and effective process for the production of low carbon chrome steel, without having recourse to highly priced raw materials nor to expensive refining operations. A low carbon chrome steel with a content of from 10 to 16% chromium is well known to possess rust resisting properties and may by my process be readily obtained from any low phosphorus pig iron having a carbon content of 4% or thereabouts. By using a substantial excess of chrome ore and by disintegrating both the pig iron and the chrome ore, so that they may be intimately intermixed before being exposed to reduction temperatures, I am able to effect a very complete decarburization of the iron.

The degree of reduction of chromium from its ore and consequently the percentage thereof finally alloyed with the steel will obviously depend on the carbon introduced by the pig iron. When a chromiferous pig iron is used the final chromium content will be increased accordingly, similarly a pig iron having a higher carbon content than that above mentioned will be susceptible of being used for the manufacture of low carbon chrome steel and chrome iron having a higher content of chromium than that specified above, or to the manufacture of low carbon ferro-chromium. In such cases, the chromium reducible from the ore to be added to the pig iron, being limited by the carbon content of the latter, the additional chromium desired in the final product must be introduced by the pig iron. This involves a supply of highly chromiferous pig iron, that is to say, richer in chromium than that obtainable in the blast furnace from natural chromiferous iron ores.

The reduction of chrome ore in a normal blast furnace for the purpose of obtaining ferro-chromium in which the relative proportions of iron and chromium are approximately those in which they exist in natural chromite is not economically possible. This is partly due to the fact that the reduction temperature of chromic oxide exceeds the normal hearth temperature of the blast fur-

nace and to the fact that a normal blast furnace slag is not suitable for promoting the reduction of chromium. Hence it is customary to use an electric shaft furnace and a 5 properly constituted slag for the carbo-reduction of chrome ore.

Nevertheless, some reduction of chrome ore in a blast furnace is possible up to a limiting value of chromium to be introduced into the 10 furnace product; this value being between 20% and 30%. Therefore, when a higher content of chromium than that reducible by the carbon of the pig iron is required in my process, a pig iron that is highly chromiferous may be obtained from the blast furnace 15 by including in the furnace burden a certain proportion of chrome ore. A pig iron of this description may therefore be utilized as the base of an electric furnace charge for a process such as I have already described, contributing thereto as much as or even a greater proportion of chromium than that rendered available by decarburizing the pig iron with crushed chrome ore in the manner aforesaid. 20 Such methods of increasing the chromium content in the final alloy are entirely within the scope of my process, in view of the methods well known to the art for the reduction of chrome ore mixed with iron ore in the 25 blast furnace.

It will be obvious to those skilled in the art, that my invention is susceptible of various changes and modifications without departing from the spirit thereof and I desire 30 therefore that only such limitations shall be placed thereupon as are imposed by the prior art or as are specifically set forth in the appended claims.

Having thus described my invention, what 35 I claim as new and desire to secure by Letters Patent is:

1. A process for the manufacture of low carbon chrome steel which consists in, intimately mixing comminuted pig iron containing 40 carbon with crushed chrome ore and slag forming material, and fusing the mixture in an electric furnace, so as to effect a reduction of chromium from the ore through the influence of the carbon in the pig iron.

2. A process for the manufacture of low carbon chrome steel which consists in, granulating molten pig iron containing carbon, mixing the latter with crushed chrome ore and lime, the ore being in excess of the carbon 55 requirement, and fusing the mixture in an electric furnace, whereby the pig iron forming the base for the carbon free chrome alloy may be substantially decarburized.

3. A process for the manufacture of low carbon chrome steel which consists in, rapidly cooling molten pig iron by granulating it in water, so as to conserve its contained carbon in combination with the iron, crushing chrome ore, effecting an intimate mixture of the 60 granulated pig iron, the crushed ore and a

suitable slag producer, fusing the mass in an electric furnace to reduce chromium from the ore by the carbon in the pig iron, and refining the resulting bath of alloy steel in the normal manner.

4. A process for the manufacture of low carbon chrome steel which consists in, intimately mixing comminuted pig iron containing carbon with chrome ore and lime, submitting the mixture to a suitable reducing 70 temperature in an electric furnace, whereby chromium in the ore may be reduced by the carbon in the iron, and refining the resulting bath of chrome steel under a lime slag in the normal manner.

5. A process for the manufacture of alloys of iron and chromium substantially low in carbon which consists in, reducing a mixture of iron ore and chrome ore in a blast furnace to produce a highly chromiferous pig iron, 75 granulating the reduction product, mixing it intimately with a further quantity of crushed chrome ore and with slag forming material, charging said mixture in the solid phase into an electric furnace, maintaining therein a 80 temperature capable of promoting the oxidation of the carbon present in the reduction product by the oxides of the ore added thereto, whereby the carbon in said reduction product may be substantially replaced by chromium 85 from the added ores.

6. A process for the manufacture of low carbon steels containing chromium and another alloying element which consists in, reducing iron ore containing the second alloying element in a blast furnace so as to include this element in the pig iron, granulating the pig iron, mixing therewith crushed chrome ore and lime, charging the mixture in the solid phase into an electric furnace, 90 maintaining therein a temperature suitable for the carbo-reduction of chromium from its ore and refining the resulting bath of alloy steel in the normal manner.

7. A process for the manufacture of low carbon high chromium iron alloys, which 95 comprises mixing crushed chrome ore and slag forming material with a finely divided blast furnace product containing a reducing agent in substantial amounts and fusing the 105 mixture.

In testimony whereof I hereunto affix my signature this 14 day of April, 1926.

FRANK O. KICHLINE.

120

125

130